

## UNITED STATES PATENT OFFICE

LYMAN W. DIXON, OF MAYWOOD, ILLINOIS

## LABELING

No Drawing.

Application filed February 19, 1930. Serial No. 429,833.

The present invention relates to a method of labeling, and it particularly relates to a method of attaching labels or other designating devices to sheets of cellulosic compositions or similar materials. Much difficulty has been experienced in satisfactorily attaching labels of paper, cloth or other materials to cellulosic films such as cellophane. A great amount of the difficulty has been due to the fact that satisfactory adhesives or adhesive compositions have not been developed. The usual adhesive mixtures, such as dextrine, glue or other water soluble colloids are generally unsatisfactory and do not result in a desirable adhesive attachment of the label or designating strip to the base material.

The object of this invention is to provide an improved method of attaching labels to sheets of cellulosic materials.

Another object of this invention is to provide new and improved methods of adhesively attaching paper or cloth labels to transparent cellulosic films such as cellophane.

A further object of this invention is to provide an improved method of adhesion of general utility.

A still further object of the present invention is to provide new and more satisfactory adhesive compositions.

Other objects will appear during the course of the following specification.

In the preferred embodiment of the invention, to which it is by no means restricted, a paper or cloth label is attached to a sheet of a cellulosic compound or to a sheet of a regenerated cellulosic material by means of a colloidal mixture, which is preferably not soluble in water per se. This cellulosic film or sheet may be composed of esters or ethers of cellulose, such as cellulose nitrate, cellulose acetate or ethoxycellulose, or on the other hand it may be composed of cellulose which is first converted into the form of a compound similar to or different than those specified above and then regenerated so as to form a smooth transparent material. The adhesive attachments of the present invention are not only applicable, however, to sheets of

cellulosic material above described, but in addition are applicable to attaching labels to materials which do not form adhesive connections with the ordinary water soluble adhesive materials.

In carrying out the present invention, the back of the label is coated with a very thin layer of a natural or synthetic resinous material. For example, varnishes or solutions made from manila chips, dammar gum, copal, shellac or synthetic resins may be utilized to coat the back of the label. As a specific example of the method of application of this thin layer of adhesive material, six and one-half pounds of manila gum are dissolved in one gallon of a special cutting alcohol and the resulting solution is applied to the back of the label. It will be noted that the preferred materials for the purpose of the present invention are water insoluble adhesives.

Before applying the label provided with this backing of water insoluble adhesive to the sheet of cellophane, the resinous adhesive material is thoroughly dried. In most cases it has been found satisfactory to store the coated label for a substantial length of time, as a result of which the very thin coating of resinous material will be aged. When it becomes desirable to attach the label to the sheet of cellophane, the adhesive resinous layer is moistened with a solution of a plasticizer in a readily volatile solvent. A wide variety of plasticizers may be utilized, but preferably those plasticizers, which are also glycerol esters of fatty acids and/or which are liquid at ordinary temperatures, are applied. Plasticizers of this character are castor oil, sulfonated castor oil, boiled linseed oil, China wood oil, etc. Although many solvents have been used and many various plasticizers dissolved therein, the preferred moistening solution is composed of castor oil and ethyl alcohol, which ethyl alcohol may contain a small quantity of wood alcohol. One mixture which has been utilized very successfully is a solution of 25% castor oil and 75% alcohol, the alcohol consisting of about 95% ethyl alcohol and about 5% wood alcohol. Of course it is possible that other solvents such

as benzine, petroleum ether, etc. might also be utilized in place of or in addition to the solvents previously mentioned.

After the label has been moistened, it is then applied to the sheet of cellophane and is preferably pressed down so that there will be a close contact over the entire adhesive surface of the label. The adhesive mixture will form a very permanent tenacious connection 10 after evaporation of the solvent and will remain in a permanently sticky or gummy condition. The adhesive connection is particularly satisfactory when oils such as castor oil, linseed oil and/or China wood oil are 15 utilized, since these materials will form a very flexible but tough adhesive connection by combination with the resinous materials.

It is obvious that many changes, variations and modifications may be made in the present invention without changing the essence 20 thereof.

What is claimed is:

1. A method of adhesively attaching a paper label to a sheet of cellophane, which 25 comprises coating the back of the label with a solution of manila gum in alcohol, permitting the alcohol to evaporate, moistening the residual resinous layer with a solution of castor oil in alcohol, and applying the moistened label to a sheet of cellophane.
2. A method of labeling which comprises placing a water insoluble resinous material upon the back of a label, drying said material, moistening the said dried material with a 35 plasticizer solution and then applying the label.
3. A method of adhesively attaching a paper label to a sheet of cellophane, which 40 comprises coating the back of the label with a solution of a resinous material in a volatile solvent, permitting the solvent to evaporate, moistening the residual resinous layer with a solution of a plasticizer in a volatile solvent, and applying the moistened label to 45 a sheet of cellophane.

In testimony whereof I have subscribed my name to the foregoing specification and claims.